# EUROPEAN PATENT SPECIFICATION

(11) **EP 1 635 365 B1**
(45) Date of publication and mention of the grant of the patent: **03.12.2008**
(21) Application number: 04405563.0
(22) Date of filing: 09.09.2004
(51) Int. Cl.: H01F 27/32, H01F 41/12, C08G 73/06, H01B 3/30

(54) **Dry-type encapsulated transformer coils**
Verkapselter Trockentransformatorwicklung
Enroulement encapsulé d'un transformateur à sec

(43) Date of publication of application: 15.03.2006
(73) Proprietor: ABB Research Ltd., 8050 Zürich (CH)
(72) Inventor: Schaal, Stéphane, 67640 Lipsheim (FR); Ghoul, Cherif, 68200 Mulhouse (FR); Rocks, Jens, 8057 Zürich (CH); Johnson, Charles W., Wytheville Virginia 24382 (US)
(74) Representative: ABB Patent Attorneys

(56) References cited:
- US-A- 4 576 768
- US-A- 4 740 343
- US-A- 5 324 767
- US-A- 5 385 989

## Description

### Field of the Invention

The present invention relates to dry-type transformers, especially dry-type distribution transformers, wherein the transformer coils are encapsulated with a cured mineral filler containing cyanate ester resin composition, and optionally is a cured mineral filler containing epoxy modified cyanate ester resin composition.

### State of the Art

Dry-type transformers are known and described e.g. in EP 0 923 785 or WO 03/107364. The dry-type transformers of the present invention contain windings that can be used as dry-type transformer high- and low-voltage windings. Dry-type transformers are used for distributing electrical energy, preferably within the range of 5 kVA to 2500 kVA. Dry-type transformers or dry-type distribution transformers comprise coils resp. windings that are generally embedded into a thermosetting insulating material. Most commonly, the insulating material is a filled epoxy resin and the windings are manufactured by vacuum casting.

Epoxy resins present a number of advantages over other thermosetting polymers. They have generally a low price, are easy to process and have good dielectrical and mechanical properties. However, epoxy resins have generally limited temperature stability. Today's market requires that transformers have an increased overload capacity and an extended lifetime. It is further required that the transformers are operated at elevated temperatures and therefore, the insulation material must exhibit an improved temperature resistance. This problem is described for example in G. Pritchard, Developments in Reinforced Plastics, vol. 5, Applied Science (1986), where it is shown that epoxy resins are not suitable for application at elevated temperatures, especially from a thermal point of view. Other technologies were developed, but these have other disadsantages compare to traditional coils encapsulated with an epoxy resin wherein the windings are manufactured by vacuum casting, especially with regard to processing and material costs. Consequently, there is a need for improved materials which are useful for encapsulating transformer coils, resp. transformer windings, which have an improved temperature stability compared to epoxy resins and further are compatible with a conventional vacuum casting manufacturing technique. Cyanate ester compositions optionally modified with one or more epoxy resins are known. However, the use of these compounds as insulation system for transformer coils in dry-type transformers has not been described.

The document US 4,576,768 discloses a dry-type transformer, wherein the transformer coils are encapsulated with a cured mineral filler containing epoxy modified isocyanate resin composition.

US 5,324,767 discloses a thermosetting resin composition which can be an isocyanate-curing epoxy resin composition containing a defined filler material for casing high-voltage coils. This reference refers to polyepoxide-polyisocyanate resins but not to polyepoxide-polycyanate ester resins. US 5,385,989 refers to a thermal resistance resin dust for the use as a friction material; electrical applications are not mentioned. A good electrical insulating material, for example for high voltage coils, needs additional physical properties; a good temperature stability per se does not suffice.

### Description of the Invention

The present invention is defined in the claims. The present invention relates to dry-type transformers, especially to dry-type distribution transformers, characterized in that the transformer coils are encapsulated with a cured mineral filler containing cyanate ester resin composition, which optionally is a cured mineral filler containing epoxy modified cyanate ester resin composition, cured resin composition is obtained from a composition comprising the components (i), (ii) and optionally (iii), wherein component (i) is a cyanate ester resin, which is present within the range of 1-60% by weight, preferably within the range of 15-30% by weight, calculated to the total weight of the insulating composition; component (ii) is a mineral filler material, which is present within the range of 20-80% by weight, preferably within the range of 40-70% by weight, and preferably within the range of 50-65% by weight, calculated to the total weight of the insulating composition; and the optional component (iii) is an epoxy resin, which is present within the range of 1-50% by weight, preferably within the range of 15-30% by weight, calculated to the total weight of the insulating composition. Said encapsulating composition is further also named as cured mineral filler containing cyanate ester resin composition optionally modified with one or more epoxy resins.

The present invention also relates to a method of encapsulating the transformer coils of a dry-type distribution transformer with the non-cured composition containing the components (i), (ii) and optionally (iii), said method according to claim 20. The insulating composition encapsulating the transformer coils optionally contains further additives as explained further on.

The cyanate ester resins are known compounds and have been described in many publications. The cyanate ester resin component within the insulating composition according to the present invention is based preferably on a single-ring cyanate monomer, such as phenyl-1,3-dicyanate, phenyl-1,4-dicyanate, wherein the phenylen ring optionally is additionally substituted by a (C₁₋₄)-alkyl group or phenyl-1,3,5-tricyanate; a phenylene cyanate oligomer or polymer, wherein the phenylene rings optionally are bound together by various bridging atoms or bridging groups such as methylene, 1,1-ethylene, 2,2-propylene, oxygen, carbonyl, carbonyloxy, sulfoxyl [-S(O)₂-] or bis-methylenoxy-dimethylsilyl; a bisphenylcyanate monomer wherein the two phenyl rings optionally are bound together by various bridging atoms or groups such as methylene, 1,1-ethylene, 2,2-propylene, oxygen, carbonyl, carbonyloxy, sulfoxyl or bis-methylenoxy-dimethylsilyl; cyanate monomers based on the naphthalene and anthraquinone structures; fluoroaliphatic dicyanates; carborane dicyanate monomers, or a mixture of these compounds. Such compounds are described e.g. in I. Hamerton, Chemistry and Technology of Cyanate Ester resins, Chapter 2, Chapman & Hall, (1994), especially pages 34-55.

The cyanate ester resin component within the insulating composition according to the present invention is based preferably on the following compounds either as single compounds or as a mixture of these compounds, of formula (I) or formula (II): or formula (III):

Preferred are compounds of formula (I) wherein R is hydrogen or compounds of formula (II) wherein D = -CH₂- or -C(CH₃)₂-, or a mixture of these compounds.

Preferred epoxy resins used within the context of the present invention are aromatic and/or cycloaliphatic compounds. These compounds are known per se. Epoxy resins are reactive glycidyl compounds containing at least two 1,2-epoxy groups per molecule. Preferably a mixture of polyglycidyl compounds is used such as a mixture of diglycidyl- and triglycidyl compounds. It is possible to combine one or more of these glycidyl compounds with a cyanate ester resin component as defined above and obtain a resin composition useful as an encapsulation material as defined in the present invention. The combination of the two components is a problem of optimization only.

Epoxy compounds useful for the present invention comprise unsubstituted glycidyl groups and/or glycidyl groups substituted with methyl groups. These glycidyl compounds preferably have a molecular weight between 200 and 1200, especially between 200 und 1000 and may be solid or liquid. The epoxy value (equiv./100 g) is preferably at least three, preferably at least four and especially at about five, preferably about 4.9 to 5.1. Preferred are glycidyl compounds which have glycidyl ether- and/or glycidyl ester groups. Such a compound may also contain both kinds of glycidyl groups, e.g. 4-glycidyloxy-benzoic acidglycidyl ester. Preferred are polyglycidyl esters with 1-4 glycidyl ester groups, especially diglycidyl ester and/or triglycidyl esters. Preferred glycidyl esters may be derived from aromatic, araliphatic, cycloaliphatic, heterocyclic, heterocyclic-aliphatic or heterocyclic-aromatic dicarbonic acids with 6 to 20, preferably 6 to 12 ring carbon atoms or from aliphatic dicarbonic acids with 2 to 10 carbon atoms. Preferred are for example optionally substituted epoxy resins of formula (IV): or formula (V):

Examples are glycidyl ethers derived from Bisphenol A or Bisphenol F as well as glycidyl ethers derived from Phenol-Novolak-resins or cresol-Novolak-resins.

Cycloaliphatic epoxy resins are for example hexahydro-o-phthalic acid-bis-glycidyl ester, hexahydro-m-phthalic acid-bis-glycidyl ester or hexahydro-p-phthalic acid-bis-glycidyl ester. Also aliphatic epoxy resins, for example 1,4-butane-diol diglycidyl - ether, may be used as a component for the composition of the present invention.

Preferred within the present invention are also aromatic and/or cycloaliphatic epoxy resins which contain at least one, preferably at least two, aminoglycidyl group in the molecule. Such epoxy resins are known and for example described in WO 99/67315. Preferred compounds are those of formula (VI): n = Zero or 1

Especially suitable aminoglycidyl compound are N,N-diglycidylaniline, N,N-diglycidyltoluidine, N,N,N',N'-tetraglycidyl-1,3-diaminobenzene, N,N,N' ,N' -tetraglycidyl-1,4-diaminobenzene, N,N,N',N'-tetraglycidylxylylendiamine, N,N,N',N'-tetraglycidyl-4,4'-diaminodiphenylmethane, N,N,N',N'-tetraglycidyl-3,3'-diethyl-4,4'-diaminodiphenylmethane, N,N,N',N'-tetraglycidyl-3,3'-diaminodiphenylsulfone, N,N'-Dimethyl-N,N'-diglycidyl-4,4'-diaminodiphenylmethane, N,N,N',N'-tetraglycidyl-alfa,alfa'-bis(4-aminophenyl)-p-diisopropylbenzene and N,N,N',N'-tetraglycidyl-alfa,alfa'-bis-(3,5-dimethyl-4-aminophenyl)-p-diisopropylbenzene.

Preferred aminoglycidyl compounds are also those of formula (VII) : or of formula (VIII):

Further aminoglycidyl compounds which can be used according to the present invention are described in e.g. Houben-Weyl, Methoden der Organischen Chemie, Band E20, Makromolekulare Stoffe, Georg Thieme Verlag Stuttgart, 1987, pages 1926-1928.

Mineral filler materials for electrical applications are known. Such materials are for example glass powder, metal oxides such as silicon oxide (Aerosil, quarz, fine quarz powder), magnesium- and aluminium hydroxide [Mg(OH)₂, Al(OH)₃, AlO(OH)], titanium oxide; metal nitrides, such as silicon nitride, boron nitride and aluminium nitride; metal carbides, such as silicon carbide (SiC); metal carbonates (dolomite, CaCO₃), metal sulfates (e.g. baryte), ground natural and synthetic minerals mainly silicates, such as talcum, glimmer, kaolin, wollastonite, bentonite; calciumsilicates such as xonolit [Ca₂Si₆O₁₇ (OH)₂]; aluminiumsilicates such as andalusite [Al₂O₃-SiO₂] or zeolithe; calcium/magnesium - carbonates such as dolomite [CaMg(CO₃)₂]; and known calcium/magnesium silicate, in different powder sizes. Preferred are silicon oxide and/or aluminium oxide, xonolite, magnesium- and aluminium hydroxide, ground natural stones, ground natural and synthetic minerals derived from silicates. The filler material has preferably an average granular size within the range of 1 µm to 300 µm, preferably within the range of 5 µm to 100 µm.

The filler material may optionally be coated for example with a silane or a siloxane known for coating filler materials, e.g. dimethylsiloxanes which may be cross linked, or other known coating materials. These compounds have been published at many publications.

The silane, e.g. a trialkylsilane or a phenyldimethylsilane, or the polysiloxanes used for coating the filler material may contain reactive groups such as hydroxyl, hydrosilyl groups (≡Si-H), carboxyl groups, (C₁-C₄) alkyl-epoxy, vinyl (≡Si-CH=CH₂) or Allyl (≡Si-CH₂CH=CH₂) , and preferably have a viscosity within the range of about 0.97 mPa·s (1 cSt) to about 19'500 mPa·s (measured according to DIN 53 019 at 25°C, calculated with a density of 0.97) and may be linear, two-dimensional or three-dimensional compounds resp. compositions, a mixture of oligomeric compounds or a mixture of the named compounds.

The viscosity of these organopolysiloxanes is preferably within the range of about 0.97 mPa.s (1 cSt) to about 4900 mPa·s, preferably within the range of 2 mPa·s to 2900 mPa·s, preferably within the range of 5 mPa·s to 700 mPa·s, according to DIN 53 019 at 25°C. Preferably the polysiloxanes have an average molecular weight within the range of about 300 to 100'000, preferably about 300 to 50'000, preferably 400 to 10'000 Dalton, wherein 1 Dalton = 1U.

The filler material optionally may be present in a "porous" form. As a "porous" filler material, which optionally may be coated, is understood, that the density of said filler material is within the range of 60% to 80%, compared to the "real" density of the non-porous filler material. Such porous filler materials have a much higher total surface than the non-porous material. Said surface preferably is higher than 20 m²/g (BET m²/g) and preferably higher than 30 m²/g (BET) and preferably is within the range of 30 m²/g (BET) to 100 m²/g (BET), preferably within the range of 40 m²/g (BET) to 60 m²/g (BET). Said porous filler material may be coated with a siloxane, preferably with an organopolysiloxane which may be cross linked, with up to 50%-80% by weight, preferably from 60%-70% by weight, calculated to the total weight of the coated filler material.

The insulating composition encapsulating the transformer coils may contain further additives such as hardeners, curing agents, plasticizers, antioxidants, light absorbers, as well as further additives used in electrical applications.

Hardeners are known to be used in epoxy resins. In the present composition such hardeners are only optional. Hardeners are for example hydroxyl and/or carboxyl containing polymers such as carboxyl terminated polyester and/or carboxyl containing acrylate- and/or methacrylate polymers and/or carboxylic acid anhydrides. Useful hardeners are further cyclic anhydrides of aromatic, aliphatic, cycloaliphatic and heterocyclic polycarbonic acids. Preferred anhydrides of aromatic polycarbonic acids are phthalic acid anhydride and substituted derivates thereof, benzene-1,2,4,5-tetracarbonic acid dianhydride and substituted derivates thereof. Numerous further hardeners are from the literature.

The optional hardener can be used in concentrations within the range of 0,2 to 1,2, equivalents of hardening groups present, e.g. one anhydride group per 1 epoxide equivalent. However, within the present invention a concentration within the range of 0,2 to 0.4, equivalents of hardening groups is preferred.

Curing agents are for example tertiary amines, such as benzyldimethylamine or amine-complexes such as complexes of tertiary amines with boron trichloride or boron trifluoride; urea derivatives, such as N-4-chlorophenyl-N',N'-dimethylurea (Monuron); optionally substituted imidazoles such as imidazole or 2-phenyl-imidazole. Preferred are tertiary amines. Other curing catalyst such as transition metal complexes of cobalt(III), copper, manganese(II), zinc in acetylacetonate may also be used, e.g. cobalt acetylacetonate(III). The amount of catalyst used is a concentration of about 50 ppm - 1000 ppm by weight, calculated to the composition to be cured.

The insulating composition is made simply by mixing all the components, optionally under vacuum, in any desired sequence and curing the mixture by heating. Preferably the hardener and the curing agent are separately added before curing. The curing temperature is preferably within the range of 50°C to 280°C, preferably within the range of 100°C to 200°C. Curing generally is possible also at lower temperatures, whereby at lower temperatures complete curing may last up to several days, depending also on catalyst present and its concentration.

For encapsulating the transformer coil with the insulating composition according to the present invention, the transformer coil is placed into a mold and the insulation composition is added. It is then possible to heat the composition, e.g. by applying an electrical current to the coil to resistively heat the composition to a desired temperature and for a time long enough, optionally under the application of vacuum, to remove all moisture and air bubbles from the coil and the insulating composition. The encapsulating composition may the be cured by any method known in the art by heating the composition to the desired curing temperature.

### Examples 1 and 2

The coils, resp. windings, of a dry-type distribution transformer are encapsulated with a thermosetting insulating material made of a filler containing epoxy modified cyanate ester resin system. The electrical, mechanical and processing properties are compared with the same coils, resp. windings encapsulated with a conventional epoxy resin. As shown, the coils of the dry-type distribution transformer encapsulated with a filler containing epoxy modified cyanate ester resin system show much better properties. The recipes used are given in Table 1.

**Table 1**

| COMPONENTS | REFERENCE | Example 1 | Example 2 |
|---|---|---|---|
| epoxy resin 1 | 100 | - | 50 |
| Hardener 2 | 82 | - | - |
| Accelerator 3 | 2 | - | - |
| cyanate ester 4 | - | 100 | 50 |
| Co-catalyst 5 | - | - | 100 ppm |
| filler (silica flour) 6 | 322 | 175 | 175 |

| | | | |
|---|---|---|---|
| 1 VE4518 Comp. A supplied by Bakelite AG (new name EPR 845) 2 VE4518 Comp. B supplied by Bakelite AG (new name EPH 845) 3 VE4518 Comp. C supplied by Bakelite AG (new name EPC 845) 4 Primaset PT-15 supplied by Lonza AG 5 Cobalt acetylacetonate supplied by Shepherd 6 Millisil W12 supplied by Quarzwerke | | | |

All of the formulations of Table 1 contain the same amount of filler (63.6% wt.).
The epoxy component is a Bisphenol A/F mixture with an epoxy equivalent of 4.9-5.1 (equiv./100g).
Short term dynamic degradation was performed by heating the materials at 10°C/minute from ambient temperature to 800°C by using a thermo gravimetric analyzer (TGA). The onset of degradation was measured and reported in Table 2 shown below. The data shows that the onset of thermal degradation is higher for the formulations of the invention than for the reference. This indicates a higher thermal stability of the formulations of the invention.

It is generally accepted by those familiar with the vacuum casting process that a material with a dynamic viscosity value of 10 Pa·s or below is suitable for the mentioned process. Steady state viscosity data show that all of the materials are suitable for a casting process.

Long term thermo-oxidative ageing characteristics were also evaluated. Accelerated ageing was performed at 260°C and flexural strength (ISO 178) was measured before and after 100 and 200 hours ageing. The fraction of the remaining flexural strength after ageing was calculated. The higher that fraction, the better the resistance to thermal ageing. It is clear from Table 2 below that the invention formulations exhibit a significantly improved resistance to thermal ageing compared to the reference.

**Table 2**

| PROPERTY | REFERENCE | Ex. 1 | Ex. 2 |
|---|---|---|---|
| Onset of thermal degradation (°C) | 360 | 410 | 371 |
| Steady state viscosity at 75°C (Pa·s) | 1.0 | 2.2 | 1.4 |
| % of initial flexural strength after 100h at 260°C | 66 | 92 | 94 |
| % of initial flexural strength after 200h at 260°C | 12 | 83 | 88 |

## Claims

1. Dry-type transformer, preferably dry-type distribution transformer, wherein the transformer coils are encapsulated with a cured mineral filler, said cured mineral filler **characterized by** containing cyanate ester resin composition, optionally epoxy modified cyanate ester resin composition, wherein said cured resin composition is obtained from a composition comprising the components (i), (ii) and optionally (iii), wherein component (i) is a cyanate ester resin, which is present within the range of 1-60% by weight, calculated to the total weight of the insulating composition; component (ii) is a mineral filler material, which is present within the range of 20-80% by weight, calculated to the total weight of the insulating composition; and the optional component (iii) is an epoxy resin, which is present within the range of 1-50% by weight, calculated to the total weight of the insulating composition.

2. Dry-type transformer according to claim 1, wherein component (i) is present within the range of 15-30% by weight, calculated to the total weight of the insulating composition; component (ii) is present within the range of 40-70% by weight, and preferably within the range of 50-65% by weight, calculated to the total weight of the insulating composition; and the optional component (iii) is present within the range of 15-30% by weight, calculated to the total weight of the insulating composition.

3. Dry-type transformer according to claim 1 or 2, wherein the cyanate ester resin within the insulating composition is based on a single-ring cyanate monomer, preferably phenyl-1,3-dicyanate, phenyl-1,4-dicyanate, wherein the phenylen ring optionally is additionally substituted by an (C₁₋₄)-alkyl group or phenyl-1,3,5-tricyanate; a phenylene cyanate oligomer or polymer, wherein the phenylene rings optionally are bound together by various bridging atoms or bridging groups preferably methylene, 1,1-ethylene, 2,2-propylene, oxygen, carbonyl, carbonyloxy, sulfoxyl or bis-methylenoxy-dimethylsilyl; a bisphenylcyanate monomer wherein the two phenyl rings optionally are bound to-gether by various bridging atoms or groups preferably methyl-lene, 1,1-ethylene, 2,2-propylene, oxygen, carbonyl, carbonyloxy, sulfoxyl or bis-methylenoxy-dimethylsilyl; cyanate monomers based on the naphthalene and anthraquinone structures; fluoroaliphatic dicyanates; carborane dicyanate monomers, or a mixture of these compounds.

4. Dry-type transformer according to claim 1 or 2, wherein said cyanate ester resin component is based on the following compounds either as single compounds or as a mixture of these compounds, of formula (I) or formula (II): or formula (III):

5. Dry-type transformer according to claim 4, wherein R of formula (I) is hydrogen or wherein D of formula (II) is -CH₂- or -C(CH₃)₂-.

6. Dry-type transformer according to claim any one of the claims 1-5, wherein the optionally present epoxy resin is based on aromatic and/or cycloaliphatic reactive glycidyl compounds containing at least two 1,2-epoxy groups per molecule, preferably a mixture of polyglycidyl compounds, preferably a mixture of diglycidyl- and triglycidyl compounds.

7. Dry-type transformer according to claim 6, wherein the epoxy compound comprises unsubstituted glycidyl groups and/or glycidyl groups substituted with methyl groups, preferably having a molecular weight between 200 and 1200, preferably between 200 und 1000.

8. Dry-type transformer according to claim 6 or 7, wherein the epoxy value (equiv./100 g) of the epoxy resin is at least three, preferably at least four and especially at about five, preferably about 4.9 to 5.1.

9. Dry-type transformer according to any one of the claims 1-8, wherein epoxy resin corresponds to formula (IV): or formula (V):

10. Dry-type transformer according to any one of the claims 1-8, wherein epoxy resin is an aromatic and/or cycloaliphatic epoxy resins which contain at least one, preferably at least two, aminoglycidyl groups in the molecule, preferably corresponding to formula (VI) : or formula (VII): or of formula (VIII):

11. Dry-type transformer according to any one of the claims 1-10, wherein the mineral filler material is selected from the group comprising glass powder, metal oxides preferably silicon oxide (Aerosil, quarz, fine quarz powder), magnesium- and aluminium hydroxide [Mg(OH)₂, Al(OH)₃, AlO(OH)₂], titanium oxide; metal nitrides, preferably silicon nitride, boron nitride and aluminium nitride; metal carbides, preferably silicon carbide (SiC); metal carbonates (dolomite, CaCO₃), metal sulfates (e.g. baryte), ground natural and synthetic minerals mainly silicates, preferably talcum, glimmer, kaolin, wollastonite, bentonite; calciumsilicates preferably xonolite [Ca₂Si₆O₁₇(OH)₂]; aluminium-silicates, preferably andalusite [Al₂O₃.SiO₂] or zeolithe; calcium/magnesium carbonates, preferably dolomite [CaMg(CO₃)₂]; and known calcium/magnesium silicate, in different powder sizes.

12. Dry-type transformer according to claims 11, wherein the mineral filler material is selected from the group comprising silicon oxide, aluminium oxide, xonolite, magnesium hydroxide, aluminium hydroxide, ground natural stones, ground natural and synthetic minerals derived from silicates, preferably with an average granular size within the range of 1 µm to 300 µm, preferably within the range of 5 µm to 100 µm.

13. Dry-type transformer according to any one of the claims 1-12, wherein the mineral filler material is coated with a silane or a siloxane, preferably with a dimethylsiloxane which may be cross linked.

14. Dry-type transformer according to claim 13, wherein the silane or the siloxane contains reactive groups selected from hydroxyl, hydrosilyl groups (≡Si-H), carboxyl groups, (C₁-C₄)-alkyl-epoxy, vinyl (≡Si-CH=CH₂) or Allyl (≡Si-CH₂CH=CH₂).

15. Dry-type transformer according to claim 13, wherein the silane or the siloxane have a viscosity within the range of about 0.97 mPa•s (1 cSt) to about 19'500 mPa•s (measured according to DIN 53 019 at 25°C, calculated with a density of 0.97), preferably within the range of 0.97 mPa•s (1 cSt) to 4900 mPa•s, preferably within the range of 2 mPa•s to 2900 mPa•s, preferably within the range of 5 mPa•s to 700 mPa•s, according to DIN 53 019 at 25°C.

16. Dry-type transformer according to claim 13, wherein the polysiloxane has an average molecular weight within the range of about 300 to 100'000, preferably about 300 to 50'000, preferably 400 to 10'000 Dalton.

17. Dry-type transformer according to any one of the claims 1-16, wherein the filler material is a "porous" filler material, of which the density is within the range of 60% to 80%, compared to the real density of the non-porous filler material, preferably having a total surface higher than 20 m²/g (BET m²/g), preferably higher than 30 m²/g (BET), preferably within the range of 30m²/g (BET) to 100 m²/g (BET), preferably within the range of 40 m²/g (BET) to 60 m²/g (BET).

18. Dry-type transformer according to any one of the claims 1-17, wherein the insulating composition encapsulating the transformer coils contains further additives selected from the group comprising hardeners, curing agents, plasticizers, antioxidants, light absorbers, as well as further additives used in electrical applications.

19. Dry-type transformer according to claim 18, wherein the hardener is a known hardener for the use in epoxy resins and is present in concentrations within the range of 0,2 to 1,2, equivalents of hardening group per 1 epoxide equivalent, preferably within the range of 0,2 to 0.4, equivalents of hardening group.

20. Method of encapsulating the transformer coils of a dry-type distribution transformer according to any one of the claims 1-19, said method comprising the steps of:
- mixing the components (i), (ii) and optionally (iii) in any desired sequence, said components being as defined in any one of the claims 1-19, and
- curing the mixture,
wherein said mixing is carried out optionally under vacuum, preferably by separately adding the hardener and the curing agent to the mixture before curing, and
said curing is carried out preferably by heating the mixture to a temperature within the range of 50°C to 280°C, preferably within the range of 100°C to 200°C, or at lower temperatures up to several days, depending on the catalyst present and its concentration.

## Patentansprüche

1. Trockentransformator, vorzugsweise Trockenverteilertransformator, worin die Transformatorspulen mit einem gehärteten mineralischen Füllstoff verkapselt sind, wobei der gehärtete mineralische Füllstoff **gekennzeichnet ist durch** einen Gehalt an Cyanatesterharzzusammensetzung, gegebenenfalls epoxidmodifizierter Cyanatesterharzzusammensetzung, worin die gehärtete Harzzusammensetzung aus einer die Komponenten (i), (ii) und gegebenenfalls (iii) enthaltenden Zusammensetzung erhalten wird, worin Komponente (i) ein Cyanatesterharz ist, das im Bereich von 1-60 Gew.-%, bezogen auf das Gesamtgewicht der Isolierzusammensetzung, vorliegt; Komponente (ii) ein mineralischer Füllstoff ist, der im Bereich von 20-80 Gew.-%, bezogen auf das Gesamtgewicht der Isolierzusammensetzung, vorliegt; und die fakultative Komponente (iii) ein Epoxidharz ist, das im Bereich von 1-50 Gew.-%, bezogen auf das Gesamtgewicht der Isolierzusammensetzung, vorliegt.

2. Trockentransformator nach Anspruch 1, worin Komponente (i) im Bereich von 15-30 Gew.-%, bezogen auf das Gesamtgewicht der Isolierzusammensetzung, vorliegt; Komponente (ii) im Bereich von 40-70 Gew.-% und vorzugsweise 50-65 Gew.-%, bezogen auf das Gesamtgewicht der Isolierzusammensetzung, vorliegt und die fakultative Komponente (iii) im Bereich von 15-30 Gew.-%, bezogen auf das Gesamtgewicht der Isolierzusammensetzung, vorliegt.

3. Trockentransformator nach Anspruch 1 oder 2, worin das Cyanatesterharz in der Isolierzusammensetzung auf einem Einring-Cyanatmonomer, vorzugsweise Phenyl-1,3-dicyanat, Phenyl-1,4-dicyanat, worin der Phenylenring gegebenenfalls zusätzlich durch eine (C₁₋₄)-Alkylgruppe substituiert ist, oder Phenyl-1,3,5-tricyanat; einem Phenylencyanat-Oligomer oder -Polymer, worin die Phenylenringe gegebenenfalls durch verschiedene Brückenatome oder Brückengruppen, vorzugsweise Methylen, 1,1-Ethylen, 2,2-Propylen, Sauerstoff, Carbonyl, Carbonyloxy, Sulfoxyl oder Bis-methylenoxy-dimethylsilyl, miteinander verbunden sind; einem Bisphenylcyanat-Monomer, worin die beiden Phenylringe gegebenenfalls durch verschiedene Brückenatome oder Brückengruppen, vorzugsweise Methylen, 1,1-Ethylen, 2,2-Propylen, Sauerstoff, Carbonyl, Carbonyloxy, Sulfoxyl oder Bis-methylenoxy-dimethylsilyl, miteinander verbunden sind; Cyanat-Monomeren auf Basis der Naphthalin-und Anthrachinonstrukturen; fluoraliphatischen Dicyanaten; Carborandicyanat-Monomeren oder einer Mischung dieser Verbindungen basiert.

4. Trockentransformator nach Anspruch 1 oder 2, worin die Cyanatesterharzkomponente auf den folgenden Verbindungen, entweder als einzelne Verbindungen oder als Mischung dieser Verbindungen, der Formel (I) oder der Formel (II): oder der Formel (III): basiert.

5. Trockentransformator nach Anspruch 4, worin R der Formel (I) für Wasserstoff steht oder D der Formel (II) für -CH₂- oder -C(CH₃)₂- steht.

6. Trockentransformator nach einem der Ansprüche 1-5, worin das gegebenenfalls vorhandene Epoxidharz auf aromatischen und/oder cycloaliphatischen reaktiven Glycidylverbindungen mit mindestens zwei 1,2-Epoxidgruppen pro Molekül, vorzugsweise einer Mischung von Polyglycidylverbindungen, vorzugsweise einer Mischung von Diglycidyl- und Triglycidylverbindungen, basiert.

7. Trockentransformator nach Anspruch 6, worin die Epoxidverbindung unsubstituierte Glycidylgruppen und/oder mit Methylgruppen substituierte Glycidylgruppen, vorzugsweise mit einem Molekulargewicht zwischen 200 und 1200, vorzugsweise zwischen 200 und 1000, enthält.

8. Trockentransformator nach Anspruch 6 oder 7, worin der Epoxywert (Äquiv./100 g) des Epoxidharzes mindestens drei, vorzugsweise mindestens 4 und insbesondere etwa fünf, vorzugsweise etwa 4,9 bis 5,1, beträgt.

9. Trockentransformator nach einem der Ansprüche 1-8, worin das Epoxidharz der Formel (IV): oder der Formel (V): entspricht.

10. Trockentransformator nach einem der Ansprüche 1-8, worin es sich bei dem Epoxidharz um ein aromatisches und/oder cycloaliphatisches Epoxidharz mit mindestens einer und vorzugsweise mindestens zwei Aminoglycidylgruppen im Molekül, vorzugsweise entsprechend der Formel (VI): oder der Formel (VII): oder der Formel (VIII): handelt.

11. Trockentransformator nach einem der Ansprüche 1-10, worin der mineralische Füllstoff aus der Gruppe enthaltend Glaspulver, Metalloxide, vorzugsweise Siliciumoxid (Aerosil, Quarz, feines Quarzpulver), Magnesium- und Aluminiumhydroxid [Mg(OH)₂, Al(OH)₃, AlO(OH)₂], Titanoxid; Metallnitride, vorzugsweise Siliciumnitrid, Bornitrid und Aluminiumnitrid; Metallcarbide, vorzugsweise Siliciumcarbid (SiC); Metallcarbonate (Dolomit, CaCO₃), Metallsulfate (z.B. Baryt), gemahlene natürliche und synthetische Mineralien, hauptsächlich Silicate, vorzugsweise Talk, Glimmer, Kaolin, Wollastonit, Bentonit; Calciumsilicate, vorzugsweise Xonolit [Ca₂Si₆O₁₇(OH)₂], Aluminiumsilicate, vorzugsweise Andalusit [Al₂O₃.SiO₂] oder Zeolith; Calcium-/Magnesiumcarbonate, vorzugsweise Dolomit [CaMg(CO₃)₂] und bekanntes Calcium-/Magnesiumsilicat, in verschiedenen Pulvergrößen ausgewählt ist.

12. Trockentransformator nach Anspruch 11, worin der mineralische Füllstoff aus der Gruppe enthaltend Siliciumoxid, Aluminiumoxid, Xonolit, Magnesiumhydroxid, Aluminiumhydroxid, gemahlene Natursteine, gemahlene natürliche und synthetische Mineralien, die sich von Silicaten ableiten, vorzugsweise mit einer mittleren Korngröße im Bereich von 1 µm bis 300 µm, vorzugsweise im Bereich von 5 µm bis 100 µm, ausgewahlt ist.

13. Trockentransformator nach einem der Ansprüche 1-12, worin der mineralische Füllstoff mit einem Silan oder einem Siloxan, vorzugsweise mit einem Dimethylsiloxan, das vernetzt sein kann, überzogen ist.

14. Trockentransformator nach Anspruch 13, worin das Silan oder das Siloxan unter Hydroxyl, Hydrosilylgruppen (≡Si-H), Carboxylgruppen, (C₁-C₄)-Alkylepoxid, Vinyl (≡Si-CH=CH₂) oder Allyl (≡Si-CH₂CH=CH₂) ausgewählte reaktive Gruppen enthält.

15. Trockentransformator nach Anspruch 13, worin das Silan oder das Siloxan eine Viskosität im Bereich von etwa 0,97 mPa·s (1 cSt) bis etwa 19'500 mPa·s (gemessen gemäß DIN 53 019 bei 25°C, berechnet mit einer Dichte von 0,97), vorzugsweise im Bereich von 0,97 mPa·s (1 cSt) bis 4900 mPa·s, vorzugsweise im Bereich von 2 mPa·s bis 2900 mPa·s, vorzugsweise im Bereich von 5 mPa·s bis 700 mPa·s, gemäß DIN 53 019 bei 25°C aufweist.

16. Trockentransformator nach Ansprüche 13, worin das Polysiloxan ein mettleres Molekulargesicht im bereich von etwa 300 bis 100000 Dalton, vorzugsweise etwa 300 bis 50000 Dalton, vorzugsweise 400 bis 10000 Dalton aufweist.

17. Trockentransformator nach einem der Ansprüche 1-16, worin es sich bei dem Füllstoff um einen "porösen" Füllstoff handelt, dessen Dichte im Bereich von 60% bis 80% im Vergleich zur realen Dichte des nichtporösen Füllstoffs liegt, vorzugsweise mit einer Gesamtoberfläche von mehr als 20 m²/g (BET m²/g), vorzugsweise mehr als 30 m²/g (BET), vorzugsweise im Bereich von 30 m²/g (BET) bis 100 m²/g (BET), vorzugsweise im Bereich von 40 m²/g (BET) bis 60 m²/g (BET).

18. Trockentransformator nach einem der Ansprüche 1-17, worin die die Transformatorspulen verkapselnde Isolierzusammensetzung ferner Additive aus der Gruppe enthaltend Härter, Härtungsmittel, Weichmacher, Antioxidantien, Lichtabsorber sowie weitere bei elektrischen Anwendungen verwendete Additive enthält.

19. Trockentransformator nach Anspruch 18, worin der Härter ein bekannter Härter zur Verwendung in Epoxidharzen ist und in Konzentrationen im Bereich von 0,2 bis 1,2 Äquivalenten Härtergruppe pro 1 Epoxidäquivalent, vorzugsweise im Bereich von 0,2 bis 0,4 Äquivalenten Härtergruppe, vorliegt.

20. Verfahren zum Verkapseln der Transformatorspulen eines Trockenverteilungstransformators nach einem der Ansprüche 1-19, bei dem man:
- die Komponenten (i), (ii) und gegebenenfalls (iii) in beliebiger Reihenfolge mischt, wobei die Komponenten wie in einem der Ansprüche 1-19 definiert sind, und
- die Mischung härtet,
wobei das Mischen gegebenenfalls unter Vakuum, vorzugsweise durch separate Zugabe des Härters und des Härtungsmittels zur Mischung vor dem Härten, durchgeführt wird und
das Härten vorzugsweise durch Erhitzen der Mischung auf eine Temperatur im Bereich von 50°C bis 280°C, vorzugsweise im Bereich von 100°C bis 200°C, oder eine niedrigere Temperatur über einen Zeitraum von bis zu einigen Tagen, je nach dem vorliegenden Katalysator und seiner Konzentration, durchgeführt wird.

## Revendications

1. Transformateur à sec, de préférence transformateur de distribution à sec, dans lequel les enroulements du transformateur sont encapsulés avec une charge minérale durcie, ladite charge minérale durcie étant **caractérisée en ce qu'**elle contient une composition de résine d'ester cyanate, éventuellement une composition de résine d'ester cyanate époxy-modifiée, où ladite composition de résine durcie est obtenue à partir d'une composition comprenant les composants (i), (ii) et éventuellement (iii), où le composant (i) est une résine d'ester cyanate, qui est présente dans la plage de 1 à 60% en poids, calculé par rapport au poids total de la composition isolante ; le composant (ii) est une matière de charge minérale, qui est présente dans la plage de 20 à 80 % en poids, calculé par rapport au poids total de la composition isolante ; et le composant éventuel (iii) est une résine époxy, qui est présente dans la plage de 1 à 50 % en poids, calculé par rapport au poids total de la composition isolante.

2. Transformateur à sec selon la revendication 1, dans lequel le composant (i) est présent dans la plage de 15 à 30% en poids, calculé par rapport au poids total de la composition isolante ; le composant (ii) est présent dans la plage de 40 à 70 % en poids, et de préférence dans la plage de 50 à 65 % en poids, calculé par rapport au poids total de la composition isolante ; et le composant éventuel (iii) est présent dans la plage de 15 à 30 % en poids, calculé par rapport au poids total de la composition isolante.

3. Transformateur à sec selon la revendication 1 ou 2, dans lequel la résine d'ester cyanate dans la composition isolante est à base d'un monomère cyanate monocyclique, de préférence le phényl-1,3-dicyanate, le phényl-1,4-dicyanate, où le noyau phénylène est éventuellement en outre substitué par un groupe alkyle en (C₁₋₄), ou le phényl-1,3,5-tricyanate ; d'un oligomère ou polymère de phénylène-cyanate, où les noyaux phénylène sont éventuellement liés ensemble par divers atomes de pontage ou groupes de pontage, de préférence un groupe méthylène, un groupe 1,1-éthylène, un groupe 2,2-propylène, un atome oxygène, un groupe carbonyle, un groupe carbonyloxy, un groupe sulfoxyle ou un groupe bis-méthylénoxydiméthylsilyle ; d'un monomère bis-phénylcyanate, où les deux noyaux phényle sont éventuellement liés ensemble par divers atomes ou groupes de pontage, de préférence un groupe méthylène, un groupe 1,1-éthylène, un groupe 2,2-propylène, un atome oxygène, un groupe carbonyle, un groupe carbonyloxy, un groupe sulfoxyle ou un groupe bis-méthylénoxy-diméthylsilyle ; de monomères cyanate à base des structures naphtalène et anthraquinone ; de dicyanates fluoroaliphatiques ; de monomères carborane-dicyanate, ou d'un mélange de ces composés.

4. Transformateur à sec selon la revendication 1 ou 2, dans lequel ledit composant résine d'ester cyanate est à base des composés suivants soit en tant que composés uniques, soit en tant que mélange de ces composés, de formule (I) ou de formule (II) : ou de formule (III) :

5. Transformateur à sec selon la revendication 4, dans lequel R de la formule (I) est un atome d'hydrogène, ou dans lequel D de la formule (II) est un groupe -CH₂- ou un groupe -C(CH₃)₂-.

6. Transformateur à sec selon l'une quelconque des revendications 1 à 5, dans lequel la résine époxy éventuellement présente est à base de composés glycidyle réactifs aromatiques et/ou cycloaliphatiques, renfermant au moins deux groupes 1,2-époxy par molécule, de préférence un mélange de composés polyglycidyle, de préférence un mélange de composés diglycidyle et triglycidyle.

7. Transformateur à sec selon la revendication 6, dans lequel le composé époxy renferme des groupes glycidyle non substitués et/ou des groupes glycidyle substitués par des groupes méthyle, de préférence présentant un poids moléculaire compris entre 200 et 1200, de préférence entre 200 et 1000.

8. Transformateur à sec selon la revendication 6 ou 7, dans lequel l'indice d'époxy (équiv./100 g) de la résine époxy est d'au moins trois, de préférence d'au moins 4 et en particulier d'au moins cinq, de préférence d'environ 4,9 à 5,1.

9. Transformateur à sec selon l'une quelconque des revendications 1 à 8, dans lequel la résine époxy correspond à la formule (IV) : ou de formule (V) :

10. Transformateur à sec selon l'une quelconque des revendications 1 à 8, dans lequel la résine époxy est une résine époxy aromatique et/ou cycloaliphatique qui renferme au moins un, de préférence au moins deux groupes aminoglycidyle dans la molécule, de préférence correspondant à la formule (VI) : ou à la formule (VII) : ou à la formule (VIII) :

11. Transformateur à sec selon l'une quelconque des revendications 1 à 10, dans lequel la matière de charge minérale est choisie parmi le groupe comprenant de la poudre de verre, des oxydes métalliques, de préférence un oxyde de silicium (l'Aerosil, le quartz, la poudre fine de quartz), un hydroxyde de magnésium et d'aluminium [Mg(OH)₂, Al(OH)₃, AlO(OH)₂], l'oxyde de titane ; des nitrures métalliques, de préférence le nitrure de silicium, le nitrure de bore et le nitrure d'aluminium ; des carbures métalliques, de préférence le carbure de silicium (SiC) ; des carbonates métalliques (la dolomite, le CaCO₃), des sulfates métalliques (par exemple, la baryte), des minéraux broyés naturels et synthétiques, principalement des silicates, de préférence le talc, le mica, le kaolin, la wollastonite, la bentonite ; des silicates de calcium, de préférence la xonolite [Ca₂Si₆O₁₇(OH)₂] ; des silicates d'aluminium, de préférence l'andalusite [Al₂O₃.SiO₂] ou une zéolite ; des carbonates de calcium/magnésium, de préférence la dolomite [CaMg(CO₃)₂] ; et des silicates de calcium/magnésium connus, dans des tailles de poudre différentes.

12. Transformateur à sec selon la revendication 11, dans lequel la matière de charge minérale est choisie parmi le groupe comprenant l'oxyde de silicium, l'oxyde d'aluminium, la xonolite, l'hydroxyde de magnésium, l'hydroxyde d'aluminium, des pierres broyées naturelles, des minéraux broyés naturels et synthétiques dérivés de silicates, de préférence présentant une granulométrie moyenne dans la plage de 1 µm à 300 µm, de préférence dans la plage de 5 µm à 100 µm.

13. Transformateur à sec selon l'une quelconque des revendications 1 à 12, dans lequel la matière de charge minérale est revêtue avec un silane ou un siloxane, de préférence avec un diméthylsiloxane qui peut être réticulé.

14. Transformateur à sec selon la revendication 13, dans lequel le silane ou le siloxane renferme des groupes réactifs choisis parmi des groupes hydroxyle, des groupes hydrosilyle (≡Si-H), des groupes carboxyle, des groupes (C₁-C₄)-alkyl-époxy, des groupes vinyle (≡Si-CH=CH₂) ou des groupes allyle (≡Si-CH₂CH=CH₂).

15. Transformateur à sec selon la revendication 13, dans lequel le silane ou le siloxane présente une viscosité dans la plage d'environ 0,97 mPa·s (1 eSt) à environ 19 500 mPa·s (mesuré conformément à DIN 53 019 à 25°C, calculé avec une densité de 0,97), de préférence dans la plage de 0,97 mPa·s (1 cSt) à 4900 mPa·s, de préférence dans la plage de 2 mPa·s à 2900 mPa·s, de préférence dans la plage de 5 mPa·s à 700 mPa·s, conformément à DIN 53 019 à 25°C.

16. Transformateur à sec selon la revendication 13, dans lequel le polysiloxane présente un poids moléculaire moyen dans la plage d'environ 300 à 100 000, de préférence d'environ 300 à 50 000, de préférence de 400 à 10 000 Dalton.

17. Transformateur à sec selon l'une quelconque des revendications 1 à 16, dans lequel la matière de charge est une matière de charge « poreuse » dont la densité est dans la plage de 60 % à 80 %, par comparaison à la densité réelle de la matière de charge non poreuse, de préférence présentant une surface totale supérieure à 20 m²/g (BET m²/g), de préférence supérieure à 30 m²/g (BET), de préférence dans la plage de 30 m²/g (BET) à 100 m²/g (BET), de préférence dans la plage de 40 m²/g (BET) à 60 m²/g (BET).

18. Transformateur à sec selon l'une quelconque des revendications 1 à 17, dans lequel la composition isolante encapsulant les enroulements du transformateur contient des additifs supplémentaires choisis parmi le groupe comprenant des agents de durcissement, des agents de traitement, des agents plastifiants, des agents anti-oxydants, des agents photoabsorbants, ainsi que des additifs supplémentaires utilisés dans des applications électriques.

19. Transformateur à sec selon la revendication 18, dans lequel l'agent de durcissement est un agent de durcissement connu pour l'utilisation dans des résines époxy et est présent en des concentrations dans la plage de 0,2 à 1,2 équivalent de groupe durcisseur pour 1 équivalent d'époxyde, de préférence dans la plage de 0,2 à 0,4 équivalent de groupe durcisseur.

20. Procédé d'encapsulation des enroulements du transformateur d'un transformateur de distribution à sec selon l'une quelconque des revendications 1 à 19, ledit procédé comprenant les étapes consistant à :
- mélanger les composants (i), (ii) et éventuellement (iii) dans une séquence souhaitée quelconque, lesdits composants étant tels que définis dans l'une quelconque des revendications 1 à 19, et
- traiter le mélange,
où ledit mélangeage est effectué éventuellement sous vide, de préférence en ajoutant séparément l'agent de durcissement et l'agent de traitement au mélange avant le traitement, et
ledit traitement est effectué de préférence en chauffant le mélange jusqu'à une température dans la plage de 50°C à 280°C, de préférence dans la plage de 100°C à 200°C, ou à des températures inférieures pendant jusqu'à plusieurs jours, en fonction du catalyseur présent et de sa concentration.
